# EUROPEAN PATENT SPECIFICATION

(11) **EP 1 859 879 B1**
(45) Date of publication and mention of the grant of the patent: **05.05.2010**
(21) Application number: 06729183.1
(22) Date of filing: 15.03.2006
(51) Int. Cl.: B22D 27/08

(54) **METHOD OF CASTING AND CASTING APPARATUS**
VERFAHREN ZUM GIESSEN UND GIESSVORRICHTUNG
METHODE DE COULAGE ET APPAREIL DE COULAGE

(30) Priority: 15.03.2005 JP 2005072732
(43) Date of publication of application: 28.11.2007
(73) Proprietor: THE JAPAN STEEL WORKS, LTD., Tokyo 100-8456 (JP); HONDA MOTOR CO., LTD., Tokyo 107-8556 (JP)
(72) Inventor: IENAGA, Yuuichi, itama, 3510193 (JP); TSUKEDA, Tadayoshi, uroran-shi, Hokkaido, 0518505 (JP); YAMADA, Hitohisa, uroran-shi, Hokkaido, 0518505 (JP); MURO, Masahiko, uroran-shi, Hokkaido, 0518505 (JP); AOKI, Yasuhiro, uroran-shi, Hokkaido, 0518506 (JP)
(74) Representative: Grünecker, Kinkeldey, Stockmair & Schwanhäusser Anwaltssozietät
(86) International application number: PCT/JP2006/305162
(87) International publication number: WO 2006/098382

(56) References cited:
- EP-A- 0 293 961
- GB-A- 1 472 288
- JP-A- 55 126 345
- JP-A- 55 126 345
- JP-A- 2000 343 204
- JP-A- 2002 331 352
- JP-A- 2002 331 354
- US-A- 2 116 367

## Description

### TECHNICAL FIELD

This invention relates to a casting method and casting apparatus suitable for casting an alloy which is subject to segregation during solidification.

### BACKGROUND ART

A casting method as defined in the preamble of claims 1 and 2 and a casting apparatus having the features as specified in the preamble of claims 5 and 6, respectively, is known from JP 2002-331352 A.
EP 0 293 961 A discloses a method and an apparatus for casting of components requiring equiaxed grain structure and low porosity and having widely different section thicknesses. The method comprises the steps of filling a mould of molten metal in a first chamber, withdrawing the filled mould into a second chamber, isolating the second chamber from the first chamber with regard to pressure, pressurizing the second chamber with a fluid up to a maximum pressure of 7 MPa and oscillating the filled mould whilst under pressure until at least partial solidification has occurred. The oscillation is performed about a ram axis at a frequency in a range of 5 to 500 cycles per minute and an amplitude in the range of 5 to 360° or greater than one complete revolution. The casting apparatus is comprised of a casting mould receiving and solidifying a molten metal, a rotary device being capable of rotary driving the casting mould in opposing directions with a vertical axis as a rotary shaft, and a rotation controlling portion controlling the rotary device to repeat specific operations including rotating the casting mould at a predetermined rotary speed in one direction for a predetermined period of time and after the predetermined period of time has lapsed, rotate the casting moulds at a predetermined rotary speed in a direction opposite to the one direction for a predetermined period of time.
US 2,116,367 A discloses an apparatus for imparting rotational oscillation and an apparatus for vibrating molten metal at high velocity. The apparatus comprises a mould secured to a table supported on a frame. Said frame is connected to a rotary shaft surrounded partially by spools of an electric motor. Moreover, a spring is connected to said shaft with one end and with the other end on an inner surface side of a case surrounding said shaft and said spring. By means of the electric motor, the mould is rotated counter-clockwise, thereby the spring is wound up. At a position of the spools in which the alternating current command is to decrease, the restoring force of the spring rotates the shaft in a clockwise direction until the alternating current passes through zero and again, increases in the reverse direction. As a consequence of said actions, an oscillatory or reciprocating rotation of the shaft is obtained.
GB 1 472 288 A relates to a method of producing metal ingots with a dense and homogeneous fine-grain structure and a reduced number of defects, such as crystallization in layers, bright borders and carbonitride segregations. Said method is comprised of steps of charging a space within a mould with molten metal obtained by melting a metal stock within the mould and allowing the metal to cool while imparting reciprocating rotary motion to said mould and to the outer solidified layer of said ingot which is in contact therewith, with respect to the molten ingot metal, through an angle of rotation ranging within 5 to180° at a reversal frequency of from 1 to 300 cycles per minute.
JP 55-126345 A discloses a casting method of large-sized killed steel ingot of superior internal characteristics and less center segregation, wherein the mold is rotated during pouring of molten steel in the mold or upon ending of the pouring and just before the rotation speed of the unsolidified molten steel synchronizes with the mold, the mold is rapidly stopped or rotated reverse. This operation is repeated at a rate of once or more in 15 minutes until the molten steel solidifies.
For alloys which are subject to weight segregation due to incorporation of additive elements having a great difference in specific gravity or alloys containing elements which are segregation during solidification, it has been desired to effectively prevent occurrence of segregation during casting in order to improve product quality. In particular, Mg alloys and other light alloys are subject to the aforementioned segregation.
Referring to segregation of alloying elements that occurs during casting, a method can be proposed which includes lowering a casting temperature in order to reduce a time required until solidification, eliminate crystal growth or prevent phases having a high specific gravity or elements having a great atomic weight from settling. However, in actual casting, fluidity of molten metal in a thick shape or complicated shape must be taken into account. Thus it is difficult to substantially lower the casting temperature. Further, in a simple shape such as ingot, the casting temperature can be lowered. However, such a material is normally thick and thus needs a long solidification time even if the casting temperature is somewhat lowered. Thus, segregation occurs inevitably.

Besides this method, a method has been proposed which comprises eliminating segregation or finely dividing texture during casting to indirectly eliminate segregation (e.g., Patent Documents 1, 2).
The method disclosed in Patent Document 1 is a casting method which comprises effecting solidification in a horizontal direction in a directional solidification furnace having a chilling plate and a heating furnace while being slowly rotated on a horizontal axis. Thereby, casting defectives such as shrinkage cavity and segregation are eliminated while providing a sufficient temperature gradient.
Further, the method disclosed in Patent Document 2 is a casting method which comprises repeating mincingly rotation/reversed rotation or rotation in one direction and suspension of rotation of a casting mold placed on a chilling plate (water-cooling plate) so that a horizontal vibration is given to the casting mold in order to produce a fine regular system structure.
Patent Document 1: JP-A-2000-343204
Patent Document 2: JP-A-2002-331354

### DISCLOSURE OF THE INVENTION

### PROBLEMS THAT THE INVENTION IS TO SOLVE

However, the casting method disclosed in Patent Document 1 is a method capable of producing cast free of cast defectives such as shrinkage cavity only when a high temperature gradient is given by using an expensive device including a chilling plate and a heating furnace. Thus, it may be difficult to apply this method to casting of ordinary low cost light alloys. Further, this method is to rotate the casting mold very slowly such that directional solidified structure and monocrystalline structure cannot be destroyed. Thus, this method is only effective when solidification speed is very low in such a case that solidifying the casting mold while heating the casting mold. However, this method cannot exert its effect on ordinary casting.

Further, the casting method disclosed in Patent Document 2 is a method which keeps a soundness of the casting material by using a chilling plate and a heating furnace as in Patent Document 1 in order to eliminate microporosity and thus requires the occupation of this device over an extended period of time. Thus, this method increases in cost. Moreover, when this temperature gradient is vertically great, it is very likely that vertical formulation segregation can occur although an effect of finely dividing the casting material can be exerted. Besides these methods, a method has been proposed which agitates the molten metal using an electromagnetic agitator to homogenize the molten metal. However, this method is disadvantageous in that it requires a huge equipment investment that adds to production cost.

The present invention has an object of providing a casting method and casting apparatus capable of giving a sufficient agitating force to molten metal without requiring the aforementioned cost of facilities, steps, etc. and hence preventing segregation to obtain a cast having an excellent quality. Another object of the present invention is to prevent the coarsening of the crystalline texture. In particular, the present invention has an object of providing a casting method and casting apparatus most suitable for the production of cast subject to segregation or ingot to be plastically worked (extrusion or forging/rolling).

### MEANS FOR SOLVING THE PROBLEMS

The above objective is achieved by a casting method as specified in claims 1 and 2 and by a casting apparatus as defined in claims 5 and 6, respectively.
Preferred embodiments of the inventive method and of the inventive apparatus are subject to the dependent claims 3, 4 and 7 to 9, respectively.

In other words, according to the present invention, by repeating the continuous rotation of the casting mold and the switch of the direction of rotation of the casting mold, the molten metal in the casting mold can be shaken without roughening the surface of the molten metal and is positively agitated. In this manner, distribution of temperature of the molten metal in the casting mold becomes uniform so that the temperature of the molten metal is uniform except the region in the vicinity of the wall of the casting mold, which is greatly affected by the cooling of the casting mold. Thus, the entire molten metal in liquid phase can be kept until the temperature thereof reaches close to the solidification starting temperature. Solidification does not begin soon after pouring but proceeds only when the temperature of the liquid crystal which has been continuously agitated falls and reaches close to the solidification starting temperature. Therefore, there is little time difference between solidification of the periphery and solidification of the central part, allowing solidification with extremely little segregates which can easily be concentrated to the final solidification site. Further, even when some segregation occurs, production of crystal nuclei is accelerated by the agitation and the size of crystalline texture becomes small. Hence, segregates produced at the grain boundary are divided more finely than ordinary, giving little effect of deteriorating strength. Moreover, not only the aforementioned segregation due to difference in melting point or degree of solid solution occurring at the grain boundary or between dendrites (branched crystal) but also weight segregation can be eliminated by the agitating effect and the solidification in a short period of time because solidification is effected with stirring to cause little settling of phase containing additive elements having a high atomic weight. Thus, by eliminating the texture which is partly low in the strength due to segregation, a good stable material having little strength dispersion can be produced. Further, secondary effects such as strength enhancement by fine division of crystal grains with agitation can be expected.

On the other hand, when no agitation is effected, the molten metal in the casting mold is given a temperature gradient from the periphery of the cast toward the central part of the cast, and the solidification is successively progressed shortly after pouring. Hence, difference in time required until the termination of solidification between the periphery and the central part thereof becomes large. Thus, as the molten metal solidifies slowly from the wall of the casting mold toward the central part of the casting mold, the texture becomes coarse. As a result, also due to prolonged solidification time, segregation is increased.

The aforementioned action normally has a greater effect as the casting material has a larger volume and thus needs a longer solidification time. When a casting material has a large volume, in order to efficiently agitate at a low rotary speed, the interior of the riser portion is preferably provided with an agitating portion given a shape allowing the agitation of the molten metal. The agitating portion may be arbitrary so far as the molten metal can be given an agitating effect and may be composed of raised portion, protrusion, agitating plate or the like. It is more effective that protrusions be provided along the vertical direction on the riser portion. The protrusions protrude beyond the liquid phase of the sprue by from about 10 mm to 25 mm after casting. Further, a plurality of the protrusions can be provided apart from each other at an interval in the circumferential direction. Preferably, the protrusions are provided in a number of one to four apart from each other at an equal angular interval. When the number of the protrusions increases, the agitating effect is eliminated. Therefore, the number of the protrusions is preferably four or less. The protrusions may be provided along the vertical direction. The protrusions may be provided obliquely to the vertical direction instead of vertical direction. The alignment of the protrusions is not limited to straight line.

Further, when the inner surface of the riser portion is in the form of a non-rotating body such as polygon, turbulence can easily occur in the interior of the riser portion when the casting mold is rotated, and agitating effect can be enhanced. On the other hand, the casting portion needs to cause entire flow and thus preferably has an inner surface in the form of a rotating body.

The rotation of the aforementioned casting mold is preferably effected at a peripheral speed of from 400 to 1,000 mm/sec on the outermost circumference of the molten metal and the time interval between the rotation in one direction and in the other direction is preferably from 5 to 50 seconds. When the aforementioned peripheral speed falls below 300 mm/sec, the molten metal in the vicinity of the wall of the casting mold, which is greatly affected by cooling, cannot be given a sufficient agitating effect. On the other hand, when a peripheral speed exceeding 1,500 mm/sec is given, the agitating effect is too great such that the surface of the liquid phase is roughened and hence defects such as cold shut and gas catch may occur. Thus, it is preferred that the casting mold be rotated at a speed falling within the aforementioned range. Further, when the time interval between the rotation in one direction and in the other direction falls below 5 seconds, the switch of direction of rotation is so frequent that sufficient rise in the flow rate cannot be obtained. On the other hand, when the time interval between the rotation in one direction and in the other direction exceeds 60 seconds, the molten metal continues to be rotated in a steady state such that it makes impossible to obtain the agitating effect efficiently. Accordingly, the aforementioned time interval of switching is thus desirable.

Further, the rotation of the casting mold preferably begins when the temperature falls within the range of from not lower than the solidification starting temperature to not higher than (solidification starting temperature + 200°C) and continues until the temperature reaches not higher than the solidification ending temperature. Since the effect of rotation of the casting mold is to uniformalize the composition and temperature distribution by agitation of the liquid phase portion, the rotation of the casting mold needs to be effected between shortly after the starting of solidification and the ending of solidification in which the liquid phase is eliminated. It is preferable to continue the rotation during this period. Referring to the timing of starting of rotation, rotation preferably begins at a time of pouring if possible, or at least before a time at which the casting portion reaches the solidification starting temperature. Referring to ending of rotation, when the rotation of the casting mold is terminated at a temperature higher than the solidification ending temperature, the distribution of temperature of the molten metal in the unsolidified region becomes ununiform such that segregation may be occurred. Thus, the rotation of the casting mold preferably continues until the temperature reaches a temperature lower than the solidification ending temperature.

The rotation of the casting mold and the switch of direction of rotation can be carried out by a rotation controlling portion which controls a rotary device composed of motor or the like. The rotation controlling portion can be composed of a control circuit, CPU which operates as programmed, etc.

The present invention is suitable for the casting of an alloy which is subject to weight segregation or segregation during solidification and can be applied particularly to Mg alloy containing zinc, rare earth metal, etc. or other light alloys. In particular, the present invention is suitable for thick cast or suitable for billet or ingot to be extruded, rolled or forged. However, the object to which the present invention can be applied is not limited to specific metallic materials but can be any metallic material which is advantageous when subjected to inhibition of segregation or fine division of texture.

### ADVANTAGE OF THE INVENTION

As mentioned above, in accordance with the casting method of the present invention, production of segregates can be minimized and a fine homogenous structure can be obtained. Accordingly, it makes possible to obtain a metallic material excellent in ductility and strength.

Further, the casting apparatus of the present invention allows a control of the rotation of the casting mold to assure the aforementioned effect.

### BRIEF DESCRIPTION OF THE DRAWINGS

[Fig. 1] Fig. 1 is a schematic diagram illustrating a casting apparatus according to an embodiment of the present invention.
[Fig. 2] Fig. 2 is a schematic diagram illustrating a modification of the same casting apparatus as described above.
[Fig. 3] Fig. 3 is a schematic diagram illustrating the testing device used for comparison in the examples of the present invention.
[Fig. 4] Fig. 4 is a schematic diagram illustrating a modification of the same testing device as used in the examples of the present invention.
[Fig. 5] Fig. 5 is a graph illustrating the relationship between the number of ribs and the depth of settlement in the examples of the present invention.
[Fig. 6] Fig. 6 is a graph illustrating the relationship between the number of ribs and the amount settled in the examples of the present invention.
[Fig. 7] Fig. 7 is a diagram illustrating the distribution of chemical components of the casting material when the rotary state of the casting mold is varied in the examples of the present invention.
[Fig. 8] Fig. 8 is a diagram illustrating the vertical and radial distribution of chemical components of the casting material when the rotary state of the casting mold is varied in the examples of the present invention.
[Fig. 9] Fig. 9 is a diagram illustrating the vertical and radial distribution of chemical components of the related casting material which is not rotated.
[Fig. 10] Fig. 10 is a photograph taken by observing the macrostructure of a cast of an inventive example.
[Fig. 11] Fig. 11 is a photograph taken by observing the macrostructure of a cast of a related example.
[Fig. 12] Fig. 12 is a view diagrammatically illustrating photographs taken by observing the macrostructure of casts of related example and inventive example.

### DESCRIPTION OF REFERENCE NUMERALS

- 1: Casting mold
- 2: Riser portion
- 6: Rotary device
- 60: Turn table
- 61: Motor
- 7: Rotation controlling portion
- 8: Agitating portion
- 11: Molten metal

### BEST MODE FOR CARRYING OUT THE INVENTION

The casting apparatus of the present invention will be described hereinafter in connection with Fig. 1. Fig. 1(a) is a schematic diagram illustrating the casting apparatus of the present invention. Fig. 1(b) is a diagram of the casting mold 1 of the casting apparatus as viewed from above.
The cylindrical casting mold 1 has a box-shaped (rectangular cylinder) riser portion 2 having a great internal dimension formed on the upper part thereof. The riser portion 2 has a carbon plate 3 stuck to the inner surface thereof for preventing the occurrence of shrinkage cavity.
The aforementioned casting mold 1 is installed on a rotary device 6 covered by an insulating material or water-cooling structure member (not shown) and the casting mold 1 is capable of being rotated by the rotary device 6. The rotary device 6 is provided with a turntable 60 on which the casting mold 1 is installed, the turntable 60 has a motor 61 attached thereto via a gear (not shown) and the turntable 60 is rotarily driven by the motor 61. The motor 61 can be adjusted for rotary speed and switched in direction of rotation.

The rotary device 6 is connected to a rotation controlling portion 7 including CPU70 and a driving circuit 71. Further, the rotation controlling portion 7 is provided with a setting portion 72 for setting the rotary speed of the casting mold and the interval between the rotation in one direction and the rotation in the other direction. The rotation controlling portion 7 is capable of preferably setting the rotary speed to from 0 to 100 rpm and the switch interval to from 1 to 300 seconds. The rotary speed setting portion may be arranged such that a proper value is inputted by operator's operation. The rotary speed setting portion may be arranged such that necessary data are previously stored in memories such as nonvolatile memory and HDD from which they are read out.

The operation of the, aforementioned casting apparatus will be described hereinafter.
Firstly, Mg alloy or the like is melted in a smelting furnace 10 such as crucible, and the molten metal 11 is then poured into the casting mold 1 through a tundish 12. The molten metal 11 is received to a predetermined height in the riser portion 2. Subsequently, a control command is given by CPU70 to the driving circuit 71 on the basis of a rotary speed and a rotation switch interval predetermined in the setting portion 72 and a control signal is given to the rotary device 6. In this manner, the rotary device 6 rotates the casting mold 1 according to the aforementioned control command. Inside the casting mold 1 which is being rotated at a proper rotary speed, an agitating effect is given such that the peripheral speed is from 400 to 1,000 mm/sec on the outermost circumference of the molten metal to uniformalize the temperature of the molten metal, and a proper turbulence occurs in the riser portion 2 to enhance the agitating effect. During this procedure, a proper rotary speed suppresses roughening of the surface of the liquid. Further, the direction of rotation of the casting mold 1 is switched at an optimum interval (5 to 60 seconds) shortly before the rotation of the casting mold 1. Therefore, the molten metal 11 can be effectively agitated the molten metal 11. In this manner, a cast having a finely divided and homogeneous structure with little segregation can be obtained.

The aforementioned embodiment has no special structure provided on the inner surface of the riser portion. However, the riser portion 2a may have an agitating portion 8 provided on the inner surface thereof for giving an agitating effect to the molten metal 11 as shown in Fig. 2. Fig. 2(a) is a schematic diagram illustrating such a casting apparatus. Fig. 2(b) is a diagram of the casting mold 1 of the casting apparatus as viewed from above. The agitating portion 8 is formed as a protrusion (rib) extending longitudinally in this embodiment. Further, the upper position of the agitating portion 8 preferably protrudes beyond the surface of the liquid when the molten metal is received in the casting mold as shown in Fig. 2(b). The protrusions are preferably disposed in a number of from one to four apart from each other at an equal angular interval in the circumferential direction. However, the present invention is not limited to a specific number of protrusions.

### EXAMPLE 1

### (Preliminary examination)

Next, in order to confirm the effect of agitation by the present invention, a preliminary examination was made to observe the behavior of water in a beaker and wax particles (specific gravity: 0.99) suspended on the water. As shown in Fig. 3, a beaker 32 having 100 wax particles 31 suspended in water 30 was placed on a turntable 33, and then rotated the turntable 33.
Rotation of the turntable 33 was made at varying rotary speeds as set forth in Table 1 and the interval of reversal of rotation was constant (10 seconds).
As a result, by adding the reversal of rotation, a good agitating effect was obtained at a predetermined rotary speed. However, an agitating force great enough to cause the wax to sink is not obtained if the process is left as it is. Then, ribs 32a as shown in Fig. 4 were provided on the inner surface of the beaker 32 at a position close to the surface of the liquid. The behavior of the wax was observed with varying numbers of sheets of rib and rotary speeds. The depth of settling of wax which had sunk most deeply is shown in Fig. 5 with the depth from the surface of the liquid to the bottom as 100%. The ratio of the amount of wax which had sunk from the surface of the liquid to the total amount is shown in Fig. 6. As a result, the more the rotary speed was, the greater is the agitating force, and the agitating effect decreased when the number of sheets of rib increased or decreased from 2, which was a peak. Further, when rotation is reversed, the agitating force reaches maximum. However, when the rotary speed is increased excessively, water is shaken more, and the molten metal can be likely roughened on the surface thereof and scattered during the actual casting.
In the case of an actual large cast, rotation may be effected at a low rotary speed so far as the peripheral speed is on the same level. Sufficient effect can be exerted when rotation is effected at about 30 rpm for φ300 mm or at about 15 rpm for φ600 mm.

**[Table 1]**

| * Results with no ribs | | | | | | |
|---|---|---|---|---|---|---|
| Rotary speed (rpm) | 40 | 60 | 80 | 100 | 120 | 140 |
| One direction | × | × | × | × | Δ | Δ |
| Opposite direction | × | × | ○ | ▲ | ▲ | ▲ |

| | | | | | | |
|---|---|---|---|---|---|---|
| ○: Wax particles rotated Δ: Became steady after rotation ▲: Liquid surface roughened ×: Wax particles moved little | | | | | | |

On the basis of the aforementioned preliminary examination, an Mg-Zn-RE alloy was casted using a casting apparatus of the aforementioned embodiment.
A casting mold made of soft steel having an inner diameter φ of 300 mm and a height of about 1,000 mm was placed on the turntable. An Mg alloy was then melted in a smelting furnace. The alloying elements were adjusted to 6.67 wt% of Y, 4.91 wt% of Zn and 1.04 wt% of La (RE) as target. The solidification starting temperature and solidification ending temperature of the alloy having this formulation are about 630°C and 500°C, respectively. The molten alloy was poured into the casting mold at a smelting temperature of 780°C. The turntable was rotated at 30 rpm (peripheral speed of 470 mm/sec on the outermost circumference) since shortly before pouring, and reversal of rotation was repeated every 35 seconds. After pouring, the casting mold was rotated for 10 minutes in total until the temperature of the casting mold reached about 470°C. The reversal of rotation was made in the shortest time at which the agitating force became steady, and the number of reversal of rotation was as many as possible until solidification. This is intended to cause vigorous agitation during reversal of rotation. Further, for comparison, casting involving no rotation was effected. The smelting method and the shape of the casting mold were the same as above. Referring to rotational condition 1, reversal was made immediately after 35 seconds, and this was repeated. Referring to rotational condition 2, rotation was suspended after 30 seconds, the molten metal was rotated by inertia for 5 seconds, reversal of rotation was made, and this was repeated.
About one hour after casting, the casting mold was detached from the device, and the cast was then withdrawn from the casting mold for analysis of components. The results are shown in Fig. 7.

In the product portion, there are observed several stationary materials (symbol ×) having components in an amount exceeding the target range. In contrast, materials which had been rotated have components in an amount falling within the target range and it is made obvious that a good formulation had been obtained. Referring to the width of dispersion, the ordinary stationary casting materials which had not been rotated showed a great dispersion, while those which had been solidified with stirring by rotation showed little variation width and became stable.

Further, the difference in the formulation of the central part and in the radial direction on the surface between the casting materials which had been stirred by rotation and the stationary casting materials was also confirmed. These are shown in Figs. 8 and 9. The rotary casting materials of Fig. 8 show formulation within the target range both in the vertical direction and in the radial direction of the cast. On the contrary, in the stationary casting materials of Fig. 9, the concentration of La, Zn and Y increase and deviate from the target range from the bottom of the cast toward the upper part thereof, at which solidification occurs late, and toward the radially central part thereof. Namely, the effect of agitation of the present invention is made obvious.
Further, the cast structure was also observed. As can be seen in the microphotograph of Fig. 10, the cast of an inventive example obtained with stirring by rotation under the rotational condition 1 has a homogeneous regular system structure. On the other hand, the cast of a comparative example obtained by stationary casting involving no agitation shows no regular system but a directional structure extending upward from the bottom as shown in the microphotograph of Fig. 11. Therefore, this cast shows a large crystal particle diameter and some gravity segregation and grain boundary segregation. Incidentally, Fig. 12 diagrammatically depicts the aforementioned microphotograph. Fig. 12 (a) is a view diagrammatically illustrating the microphotograph of the cast of comparative example shown in Fig. 11. Fig. 12(b) is a view diagrammatically illustrating the microphotograph of the cast of inventive example shown in Fig. 10.
While the present invention has been described in detail and with reference to specific embodiments thereof, it will be apparent to one skilled in the art that various changes and modifications can be made therein without departing from the subject matter defined by the claims.

### INDUSTRIAL APPLICABILITY

Based on the casting method of the present invention, the production of segregates can be minimized and a fine homogenous structure can be obtained. Accordingly, it makes possible to obtain a metallic material excellent in ductility and strength.
Further, the casting apparatus of the present invention allows the control of the rotation of the casting mold to assure the aforementioned effect.

## Claims

1. A casting method comprising:
rotating a casting mold (1) having a molten metal (11) received therein in one direction on a vertical axis as a rotary shaft for a predetermined period of time while solidifying the molten metal (11);
after lapsing the predetermined period of time, rotating the casting mold(1) in a direction opposite to the one direction for a predetermined period of time; and
repeating the rotations of the casting mold (1) in opposing directions to solidify the molten metal (11),
**characterized in that**
the inner surface of the riser portion (2) of the casting mold (1) has a shape of a non-rotating body, and the inner surface of the casting portion of the casting mold (1) has a shape of a rotating body for providing the molten metal (11) in the casting mold(1) with an agitating force in accordance with a rotation of the casting mold (1).

2. A casting method comprising:
rotating a casting mold (1) having a molten metal (11) received therein in one direction on a vertical axis as a rotary shaft for a predetermined period of time while solidifying the molten metal (11);
after lapsing the predetermined period of time, rotating the casting mold (1) in a direction opposite to the one direction for a predetermined period of time; and
repeating the rotations of the casting mold (1) in opposing directions to solidify the molten metal (11),
**characterized in that**
the inner surface of the casting portion of the casting mold (1) has a shape of a rotating body and the inner surface of the riser portion (2a) of the casting mold (1) has a shape of a rotating body, wherein the inner surface of the riser portion (2a) being provided with an agitating portion (8) for providing the molten metal in the casting mold (1) with an agitating force in accordance with a rotation of the casting mold (1), the agitating portion (8) being formed as a protrusion extending longitudinally.

3. The casting method according to claim 1 or 2,
wherein the rotations of the casting mold(1) are effected at a peripheral speed of from 400 to 1,000 mm/sec on an outermost circumference of the molten metal(11), and
wherein rotation time for one direction of the rotations is 5 to 60 seconds.

4. The casting method according to any one of claims 1 to 3,
wherein the rotations of the casting mold(1) in opposing directions begin when a temperature falls within a range of from not lower than a solidification starting temperature of the molten metal (11) to not higher than (solidification starting temperature + 200 deg. C), and
wherein the method continues the rotations until a solidification is completed.

5. A casting apparatus comprising:
a casting mold (1) that receives and solidifies a molten metal(11);
a rotary device (6) that is capable of rotary driving the casting mold (1) in opposing directions with a vertical axis as a rotary shaft; and
a rotation controlling portion (7) that controls the rotary device (6) to repeat operations including:
continuously rotate the casting mold(1) at a predetermined rotary speed in one direction for a predetermined period of time; and
after the predetermined period of time is lapsed, continuously rotate the casting mold (1) at a predetermined rotary speed in a direction opposite to the one direction for a predetermined period of time,
**characterized in**
**that** the inner surface of the riser portion (2) of the casting mold (1) has a shape of a non-rotating body, and the inner surface of the casting portion of the casting mold (1) has a shape of a rotating body for providing the molten metal (11) in the casting mold (1) with an agitating force in accordance with a rotation of the casting mold (1).

6. A casting apparatus comprising:
a casting mold (1) that receives and solidifies a molten metal (11);
a rotary device (6) that is capable of rotary driving the casting mold (1) in opposing directions with a vertical axis as a rotary shaft; and
a rotation controlling portion (7) that controls the rotary device (6) to repeat operations including:
continuously rotate the casting mold (1) at a predetermined rotary speed in one direction for a predetermined period of time; and
after the predetermined period of time is lapsed, continuously rotate the casting mold (1) at a predetermined rotary speed in a direction opposite to the one direction for a predetermined period of time,
**characterized in**
**that** the inner surface of the casting portion of the casting mold (1) has a shape of a rotating body and the inner surface of the riser portion (2, 2a) of the casting mold (1) has a shape of a rotating body, wherein the inner surface of the riser portion (2, 2a) being provided with an agitating portion (8) for providing the molten metal (11) in the casting mold with an agitating force in accordance with a rotation of the casting mold (1), the agitating portion (8) being formed as a protrusion extending longitudinally.

7. The casting apparatus according to claim 6, wherein the agitating portion (8) includes a protrusion formed along the vertical direction on the inner surface of the riser portion (2, 2a).

8. The casting apparatus according to claim 7,
wherein the protrusion has an upper end high enough to protrude beyond a sprue.

9. The casting apparatus according to claim 7 or 8,
wherein the protrusion is provided in a number of from one to four with an interval in a circumferential direction therebetween.

## Patentansprüche

1. Gießverfahren, das umfasst:
Drehen einer Gießform (1), in der ein geschmolzenes Metall (11) aufgenommen ist, in einer Richtung auf einer vertikalen Achse als einer Drehwelle über einen vorgegebenen Zeitraum, während das geschmolzene Metall (11) verfestigt wird;
nach Ablauf des vorgegebenen Zeitraums Drehen der Gießform (1) in einer Richtung entgegengesetzt zu der einen Richtung über einen vorgegebenen Zeitraum; und
Wiederholen der Drehungen der Gießform (1) in einander entgegengesetzten Richtungen, um das geschmolzene Metall (11) zu verfestigen,
**dadurch gekennzeichnet, dass**
die Innenfläche des Speiseabschnitts (2) der Gießform eine Form eines nicht rotierenden Körpers hat und die Innenfläche des Gießabschnitts der Gießform (1) eine Form eines rotierenden Körpers hat, um entsprechend einer Drehung der Gießform (1) eine Rührkraft auf das geschmolzene Metall (11) in der Gießform (1) auszuüben.

2. Gießverfahren, das umfasst:
Drehen einer Gießform (1), in der ein geschmolzenes Metall (11) aufgenommen ist, in einer Richtung auf einer vertikalen Achse als einer Drehwelle über einen vorgegebenen Zeitraum, während das geschmolzene Metall (11) verfestigt wird;
nach Ablauf des vorgegebenen Zeitraums Drehen der Gießform (1) in einer Richtung entgegengesetzt zu der einen Richtung über einen vorgegebenen Zeitraum; und
Wiederholen der Drehungen der Gießform (1) in einander entgegengesetzten Richtungen, um das geschmolzene Metall (11) zu verfestigen,
**dadurch gekennzeichnet, dass**
die Innenfläche des Gießabschnitts der Gießform (1) eine Form eines rotierenden Körpers hat und die Innenfläche des Speiseabschnitts (2a) der Gießform (1) eine Form eines rotierenden Körpers hat, wobei die Innenfläche des Speiseabschnitts (2a) mit einem Rührabschnitt (8) versehen ist, um entsprechend einer Drehung der Gießform (1) eine Rührkraft (8) auf das geschmolzene Metall in der Gießform (1) auszuüben, und der Rührabschnitt (8) als ein Vorsprung ausgebildet ist, der in Längsrichtung vorsteht.

3. Gießverfahren nach Anspruch 1 oder 2,
wobei die Drehungen der Gießform (1) mit einer Umfangsgeschwindigkeit von 400 bis 1000 mm/s an einem Außenumfang des geschmolzenen Metalls (1) ausgeführt werden, und
wobei die Drehungszeit für eine Richtung der Drehungen 5 bis 60 Sekunden beträgt.

4. Gießverfahren nach einem der Ansprüche 1 bis 3,
wobei die Drehungen der Gießform (1) in einander entgegengesetzte Richtungen beginnen, wenn eine Temperatur in einen Bereich von Temperaturen nicht unter einer Verfestigungs-Anfangstemperatur des geschmolzenen Metalls (11) und nicht über einer Verfestigungs-Anfangstemperatur + 200 °C fällt, und,
wobei das Verfahren die Drehungen fortführt, bis eine Verfestigung abgeschlossen ist.

5. Gießvorrichtung, die umfasst:
eine Gießform (1), die ein geschmolzenes Metall (11) aufnimmt und es verfestigt;
eine Dreheinrichtung (6), die in der Lage ist, die Gießform (1) drehend in einander entgegengesetzten Richtungen mit einer vertikalen Achse als einer Drehwelle zu drehen; und
einen Drehungs-Steuerabschnitt (7), der die Dreheinrichtung (6) so steuert, dass sie die Vorgänge wiederholt, die einschließen:
kontinuierliches Drehen der Gießform (1) mit einer vorgegebenen Drehgeschwindigkeit in einer Richtung über einen vorgegebenen Zeitraum; und
wenn der vorgegebene Zeitraum abgelaufen ist, kontinuierliches Drehen der Gießform (1) mit einer vorgegebenen Drehgeschwindigkeit in einer Richtung entgegengesetzt zu der einen Richtung über einen vorgegebenen Zeitraum,
**dadurch gekennzeichnet, dass**
die Innenfläche des Speiseabschnitts (2) der Gießform (1) eine Form eines nicht rotierenden Körpers hat und die Innenfläche des Gießabschnitts der Gießform (1) eine Form eines rotierenden Körpers hat, um entsprechend einer Drehung der Gießform (1) eine Rührkraft auf das geschmolzene Metall (11) in der Gießform (1) auszuüben.

6. Gießvorrichtung, die umfasst:
eine Gießform (1), die ein geschmolzenes Metall (11) aufnimmt und es verfestigt;
eine Dreheinrichtung (6), die in der Lage ist, die Gießform (1) drehend in einander entgegengesetzten Richtungen mit einer vertikalen Achse als einer Drehwelle zu drehen; und
einen Drehungs-Steuerabschnitt (7), der die Dreheinrichtung (6) so steuert, dass sie die Vorgänge wiederholt, die einschließen:
kontinuierliches Drehen der Gießform (1) mit einer vorgegebenen Drehgeschwindigkeit in einer Richtung über einen vorgegebenen Zeitraum; und
wenn der vorgegebene Zeitraum abgelaufen ist, kontinuierliches Drehen der Gießform (1) mit einer vorgegebenen Drehgeschwindigkeit in einer Richtung entgegengesetzt zu der einen Richtung über einen vorgegebenen Zeitraum,
**dadurch gekennzeichnet, dass**
die Innenfläche des Gießabschnitts der Gießform (1) eine Form eines rotierenden Körpers hat und die Innenfläche des Speiseabschnitts (2a) der Gießform (1) eine Form eines rotierenden Körpers hat, wobei die Innenfläche des Speiseabschnitts (2a) mit einem Rührabschnitt (8) versehen ist, um entsprechend einer Drehung der Gießform (1) eine Rührkraft (8) auf das geschmolzene Metall (11) in der Gießform (1) auszuüben, und der Rührabschnitt (8) als ein Vorsprung ausgebildet ist, der in Längsrichtung vorsteht.

7. Gießvorrichtung nach Anspruch 6, wobei der Rührabschnitt (8) einen Vorsprung enthält, der in der vertikalen Richtung an der Innenfläche des Speiseabschnitts (2, 2a) ausgebildet ist.

8. Gießvorrichtung nach Anspruch 7,
wobei der Vorsprung ein oberes Ende hat, das so hoch ist, dass es über einen Einguss hinaus vorsteht.

9. Gießvorrichtung nach Anspruch 7 oder 8,
wobei der Vorsprung in einer Anzahl von eins bis vier mit einem Abstand in Umfangsrichtung dazwischen vorhanden ist.

## Revendications

1. Procédé de coulée comportant le fait de :
faire tourner un moule de coulée (1) ayant du métal fondu (11) reçu dedans dans une première direction sur un axe vertical en tant qu'arbre rotatif pendant une durée prédéterminée tout en solidifiant le métal fondu (11) ;
après l'écoulement de la durée prédéterminée, faire tournant le moule de coulée (1) dans une direction opposée à la première direction pendant une durée prédéterminée ; et
répéter les rotations du moule de coulée (1) dans des directions opposées afin de solidifier le métal fondu (11),
**caractérisé en ce que**
la surface intérieure de la partie de masselotte (2) du moule de coulée (1) a une forme d'un corps qui n'est pas de révolution, et la surface intérieure de la partie de coulée du moule de coulée (1) a une forme d'un corps de révolution afin de pourvoir le métal fondu (11) dans le moule de coulée (1) d'une force d'agitation en fonction d'une rotation du moule de coulée (1).

2. Procédé de coulée comportant le fait de :
faire tourner un moule de coulée (1) ayant du métal fondu (11) reçu dedans dans une première direction sur un axe vertical en tant qu'arbre rotatif pendant une durée prédéterminée tout en solidifiant le métal fondu (11) ;
après l'écoulement de la durée prédéterminée, faire tourner le moule de coulée (1) dans une direction opposée à la première direction pendant une durée prédéterminée ; et
répéter les rotations du moule de coulée (1) dans des directions opposées afin de solidifier le métal fondu (11),
**caractérisé en ce que**
la surface intérieure de la partie de coulée du moule de coulée (1) a une forme d'un corps de révolution et la surface intérieure de la partie de masselotte (2a) du moule de coulée (1) a une forme d'un corps de révolution, la surface intérieure de la partie de masselotte (2a) étant pourvue d'une partie d'agitation (8) afin de pourvoir le métal fondu dans le moule de coulée (1) d'une force d'agitation en fonction d'une rotation du moule de coulée (1), la partie d'agitation (8) étant sous la forme d'une saillie s'étendant longitudinalement.

3. Procédé de coulée selon la revendication 1 ou 2, selon lequel les rotations du moule de coulée (1) sont effectuées à une vitesse périphérique de 400 à 1000 mm/s sur une circonférence extérieure du métal fondu (11), et
selon lequel le temps de rotation pour la première direction des rotations est de 5 à 60 secondes.

4. Procédé de coulée selon l'une quelconque des revendications 1 à 3, selon lequel les rotations du moule de coulée (1) dans des directions opposées commencent quand une température tombent dans une plage de pas moins qu'une température de début de solidification du métal fondu (11) à pas plus qu'une (température de début de solidification + 200 degrés C), et
selon lequel le procédé continue les rotations jusqu'à ce qu'une solidification soit terminée.

5. Dispositif de coulée comportant :
un moule de coulée (1) qui reçoit et solidifie un métal fondu (11) ;
un dispositif rotatif (6) qui est capable d'entraîner en rotation le moule de coulée (1) dans des directions opposées avec un axe vertical en tant qu'arbre rotatif ; et
une partie de commande de rotation (7) qui commande le dispositif rotatif (6) afin de répéter des opérations comprenant le fait de :
faire tourner de manière continue le moule de coulée (1) à une vitesse de rotation prédéterminée dans une première direction pendant une durée prédéterminée ; et
une fois que la durée prédéterminée s'est écoulée, faire tourner de manière continue le moule de coulée (1) à une vitesse de rotation prédéterminée dans une direction opposée à la première direction pendant une durée prédéterminée,
**caractérisé en ce que** la surface intérieure de la partie de masselotte (2) du moule de coulée (1) a une forme d'un corps qui n'est pas de révolution, et la surface intérieure de la partie de coulée du moule de coulée (1) a une forme d'un corps de révolution afin de pourvoir le métal fondu (11) dans le moule de coulée (1) d'une force d'agitation en fonction d'une rotation du moule de coulée (1).

6. Dispositif de coulée comportant :
un moule de coulée (1) qui reçoit et solidifie un métal fondu (11) ;
un dispositif rotatif (6) qui est capable d'entraîner en rotation le moule de coulée (1) dans des directions opposées avec un axe vertical en tant qu'arbre rotatif ; et
une partie de commande de rotation (7) qui commande le dispositif rotatif (6) afin de répéter des opérations comprenant le fait de :
faire tourner de manière continue le moule de coulée (1) à une vitesse de rotation prédéterminée dans une première direction pendant une durée prédéterminée ; et
une fois que la durée prédéterminée s'est écoulée, faire tourner de manière continue le moule de coulée (1) à une vitesse de rotation prédéterminée dans une direction opposée à la première direction pendant une durée prédéterminée,
**caractérisé en ce que** la surface intérieure de la partie de coulée du moule de coulée (1) a une forme d'un corps de révolution et la surface intérieure de la partie de masselotte (2, 2a) du moule de coulée (1) a une forme d'un corps de révolution, la surface intérieure de la partie de masselotte (2, 2a) étant pourvue d'une partie d'agitation (8) afin de pourvoir le métal fondu (11) dans le moule de coulée d'une force d'agitation en fonction d'une rotation du moule de coulée (1), la partie d'agitation (8) étant sous la forme d'une saillie s'étendant longitudinalement.

7. Dispositif de coulée selon la revendication 6, dans lequel la partie d'agitation (8) comprend une saillie formée le long de la direction verticale sur la surface intérieure de la partie de masselotte (2, 2a).

8. Dispositif de coulée selon la revendication 7, dans lequel la saillie a une extrémité supérieure suffisamment haute pour dépasser au delà d'une masse de coulée.

9. Dispositif de coulée selon la revendication 7 ou 8, dans lequel la saillie est prévue dans un nombre de un à quatre avec un intervalle dans une direction circonférentielle entre elles.
